

United States Patent [19]  
Birke

[11] 3,867,399  
[45] Feb. 18, 1975

[54] DIBENZIMIDAZOLE-DIUREAS

[75] Inventor: August G. Birke, Godfrey, Ill.

[73] Assignee: Shell Oil Company, New York, N.Y.

[22] Filed: Aug. 9, 1973

[21] Appl. No.: 386,910

Related U.S. Application Data

[62] Division of Ser. No. 169,460, Aug. 5, 1971, Pat. No. 3,752,765.

[52] U.S. Cl. .... 260/309.2

[51] Int. Cl. .... C07d 49/38

[58] Field of Search ..... 260/309.2

[56] References Cited

UNITED STATES PATENTS

3,222,285 12/1965 Rai et al. .... 252/137  
3,752,765 8/1973 Birke ..... 252/51.5 A

Primary Examiner—Henry R. Jiles

Assistant Examiner—C. M. S. Jaisle

Attorney, Agent, or Firm—Leonard P. Miller; Henry C. Geller

[57] ABSTRACT

Dibenzimidazole-diurea compounds corresponding to the formula:



wherein R<sub>1</sub> and R<sub>2</sub> are hydrocarbyl radicals and R<sub>3</sub> is a hydrocarbylene radical, are highly efficacious grease thickening agents.

5 Claims, No Drawings

## DIBENZIMIDAZOLE-DIUREAS

This is a division of application Ser. No. 169,460, filed Aug. 5, 1971, now U.S. Pat. No. 3,752,765, patented Aug. 14, 1973.

## BACKGROUND OF THE INVENTION

## 1. Field of the Invention

This invention relates to a novel class of dibenzimidazole-diurea compounds and grease compositions gelled therewith.

## 2. Description of the Prior Art

It has become increasingly important that grease compositions be able to provide adequate lubrication

ing need for the development of thickening agents which will not only produce greases having high dropping points, but which will additionally augment other important properties of the finished product. The present invention provides such a class of thickening agents.

## SUMMARY OF THE INVENTION

It has now been found that grease compositions having excellent high temperature lubricating properties can be produced by incorporating into an oleaginous base vehicle, a minor amount of a dibenzimidazole-diurea compound corresponding to the formula:



at high temperatures, e.g., temperatures of 350°F to 450°F or higher. Numerous thickening agents have been proposed for use in such greases including soap base thickeners, inorganic clay thickeners and organic thickening agents. Examples of this latter class of thickening agents include various polyureas, ureido compounds, aminoaryl diureas, triazines and the like. Such organic thickening agents are typically prepared by reacting one or more mono-, di-, or polyamines with one or more mono-, di-, or polyisocyanates. Other related organic thickeners include arylcarbamyl compounds formed by reacting an aromatic amine with the reaction product of an aromatic diisocyanate and p-aminobenzoic acid.

While organic thickening agents of the aforementioned types produce greases having desirably high dropping points, this is but one measure of a grease's ability to perform satisfactorily at high temperatures. Other important properties include thermal and mechanical stability, high temperature bearing performance, oxidation and corrosion resistance, etc. While additives are normally incorporated into grease compositions to improve one or more of these properties, the thickening agent itself can significantly affect, either favorably or adversely, the properties of the finished grease product. Thus, in spite of the numerous organic thickening agents known in the art, there is a continu-

25  
30  
35  
wherein R<sub>1</sub> and R<sub>2</sub> are hydrocarbyl radicals and R<sub>3</sub> is a hydrocarbylene radical. (By hydrocarbyl or hydrocarbylene is meant monovalent or divalent organic radicals, respectively, comprising solely carbon and hydrogen. Such radicals may be aliphatic, acyclic or aromatic, or partially aliphatic and partially aromatic, e.g., alkaryl or aralkyl.) Not only do the grease compositions of the invention have high dropping points, but in addition they have excellent mechanical and thermal stability, and high temperature bearing performance properties as well. These excellent qualities are believed attributable in large part to the unique dibenzimidazole structure of the present thickening agents which produces an extremely stable molecule.

## DESCRIPTION OF THE PREFERRED EMBODIMENTS

40 The aforescribed dibenzimidazole-diurea thickening agents can be conveniently prepared by reacting one mole of a dicarboxylic acid or its anhydride with two moles of a nitrosubstituted phenylenediamine, followed by reduction of the nitro groups to amine groups, 45 and further reaction with two moles of a monoisocyanate. This procedure is illustrated by the following equations:

Equation 1



Equation 2



Equation 3



An alternative method of preparing the bis-nitrobenzimidazole produced in Equation 1 is to react the dicarboxylic acid or its anhydride with two moles of a phenylene diamine which is not nitro-substituted. The resultant product can be subsequently nitrated to produce the bis-nitrobenzimidazole, which is then converted to its amino form and reacted with two moles of the monoisocyanate as shown in Equations 2 and 3 above. A more detailed description of the preparation of the dibenzimidazole-diurea thickeners is given in the examples.

Dicarboxylic acids or anhydrides which can be suitably employed in preparing the thickeners of the invention include the acids or anhydrides of aliphatic dicarboxylic acids such as succinic, glutaric, adipic, pimelic, suberic, azelaic, sebatic acids or anhydrides, as well as aromatic dicarboxylic acids such as phthalic, isophthalic or terephthalic acids or anhydrides or their esters. Cyclohexanedicarboxylic acids or anhydrides are likewise suitable, e.g., 1,2- or 1,4-cyclohexanedicarboxylic acid or anhydride, and also tetrahydrophthalic acid or anhydride. Hydrocarbyl substituted dicarboxylic acid and anhydrides can also be employed, for example, alkyl- or alkenyl-substituted succinic anhydrides corresponding to the formula



wherein R is an alkyl or alkenyl substituent of from 1 to 16 carbon atoms or more. Aliphatic dicarboxylic acids or anhydrides are preferred, and in general are selected so that the R<sub>3</sub> radical of the previously depicted formula has from 2 to 20, preferably from 2 to 12 carbon atoms.

Phenylene diamines suitable for preparing the thickening agents of the invention are those having amino groups in the ortho position, i.e., o-phenylene diamines. When the thickening agents are prepared in accordance with Equation 1, o-phenylamine diamines having a nitro substituent must be employed, e.g., 4-nitro-o-phenylene diamine. In addition to the nitro substituent, o-phenylene diamines having other substituents, e.g., alkyl or halo substituents, can also be employed provided that such substituents do not appreciably interfere with the reaction of the phenylene diamine with the dicarboxylic acid or anhydride.

Phenylene diamines employed in accordance with the alternative procedure discussed above need not contain a nitro substituent since the addition of the nitro groups is accomplished subsequent to formation

of the bis-benzimidazole. Hence, when this method of preparation is employed, unsubstituted o-phenylene diamine may be utilized or any other o-phenylene diamine having substituents which will not appreciably interfere with the formation of the bis-benzimidazole intermediate or its subsequent nitration. Examples of such phenylene diamines include 4-chloro-o-phenylene diamine and 3,4-toluene diamine.

Monoisocyanates which may be employed in accordance with the invention include aliphatic monoisocyanates or aromatic monoisocyanates having at least one aliphatic substituent of eight or more carbon atoms. Preferred monoisocyanate reactants include straight or branched chain, saturated or unsaturated aliphatic monoisocyanates having from 6 to 30, and more preferably from 12 to 24, carbon atoms. Examples of such isocyanates include cyclohexyl isocyanate, octyl isocyanate, decyl isocyanate, dodecyl isocyanate, tetradecyl isocyanate, pentadecyl isocyanate, hexadecyl isocyanate, heptadecyl isocyanate, octadecyl isocyanate, octadecenyl isocyanate, eicosyl isocyanate, docosyl isocyanate, tetracosyl isocyanate and the like. Mixtures of the aforementioned isocyanates can also be employed including mixtures of saturated and unsaturated aliphatic isocyanates. Aliphatic isocyanates having 16 to 18 carbon atoms and mixtures thereof are particularly preferred. The R<sub>1</sub> and R<sub>2</sub> radicals in the aforementioned formula are derived from the monoisocyanate reactant.

The thickening agents of the invention are generally employed in grease compositions in an amount sufficient to gel the oleaginous base vehicle to grease consistency. This amount can vary, for example, from about 5-50 percent by weight of the total composition. Normally, however, thickener concentrations of 10-35 percent by weight are sufficient to impart the desired consistency of the inventive compositions.

A wide variety of lubricating oils may be employed as the base vehicle in the present compositions. Suitable base oils include mineral lubricating oils such as naphthenic base, paraffin base or mixed base oils having a viscosity in the range of from 50 SSU at 100°F to 300 SSU at 210°F; synthetic hydrocarbon oils such as oligomerized alpha-olefins and oils derived from coal products; synthetic oils such as alkylene polymers, alkylene oxide-type polymers, polyalkene glycols, polyethers, phosphate esters, dicarboxylic acid esters and pentaerythritol esters. The above oils may be used individually or in mixtures thereof, wherever miscible or made so by the use of solvents. Of the aforementioned base oils, mineral lubricating oils having viscosities of from about 400 to 700 SSU at 100°F are especially preferred.

In addition to the dibenzimidazole-diurea thickeners, the present compositions can also contain anti-

corrosion additives such as disodium sebacate, glyceryl monooleate, sodium sulfonates, sodium nitrite, aminobenzo-triazoles, and isostearamides or imidazolines of tetraethylenglypentamine; oxidation inhibitors such as phenyl-alpha-naphthylamine, phenyl-beta-naphthylamine, diphenylamines, phenothiazine, dithiocarbamates and various analogs and homologs thereof; viscosity index improvers such as methacrylate polymers and copolymers; extreme pressure agents, and any other additive recognized in the art to perform a particular function or functions.

The following examples illustrate the method of preparation of the present thickeners and their excellent properties. It is to be understood, however, that these examples are presented for illustrative purposes only and that the invention in its broader aspects should not be limited thereto.

#### EXAMPLE I

A 4-liter round bottom flask was charged with 302.2 g (2 moles) of 4-nitro-o-phenylene diamine, 100.0 g (1 mole) of succinic anhydride and 2 liters of 4-normal hydrochloric acid solution. The flask and its contents were then refluxed, with stirring, for 24 hours. Heating was discontinued and the reactants were cooled to 0°C, filtered, and the filtrate was discarded. The precipitate was collected and neutralized with 1,500 ml of 5 normal ammonium hydroxide solution, refiltered, and washed twice with water. The neutralized material resulting was dissolved in refluxing ethylene glycol, treated with decolorizing charcoal, filtered and the filtrate cooled. The crystalline precipitate that appeared was collected, washed with ethanol and dried. The yield was 65 grams of 1,2-bis(5-nitrobenzimidazoyl-2)ethane having a melting point of 305°C.

56.04 g (0.16 mole) of the above product was then suspended in 1,200 ml of 3 normal hydrochloric acid

solution to which was added palladium on charcoal catalyst and reduction of the nitro groups effected in a low pressure hydrogenation apparatus. The catalyst was then filtered off, the filtrate neutralized with sodium bicarbonate and the resulting precipitate collected. After washing with water and drying, 41.5 g of 1,2-bis(5-aminobenzimidazoyl-2)ethane was obtained having a melting point of 154°-155°C.

14.62 g (0.05 mole) of the above material was placed 10 into a 500-ml resin flask equipped with a mechanical stirrer together with 30 g (0.1 mole) of a 70:30 molar ratio octadecyl isocyanate:hexadecylisocyanate mixture in 253 g of HVI-500 Neutral oil. This suspension was heated with stirring, under nitrogen, to 127°C. 15 Upon completion of the reaction, the contents were cooled to approximately 110°C and then milled three times in a three-roll paint mill. The resulting grease had an ASTM dropping point of 510°F, and an ASTM worked penetration (60 strokes) of 272.

20

#### EXAMPLE II

A series of grease compositions containing various dibenzimidazole-diurea thickening agents in accordance with the invention were prepared employing a 25 variety of base vehicles. The reactants employed in the preparation of the respective thickeners and the properties of the grease compositions gelled therewith are presented in Table I.

30

#### EXAMPLE III

In order to demonstrate the excellent high temperature performance characteristics of dibenzimidazole-diurea-thickened grease compositions, several of the 35 greases of Example II containing conventional oxidation and corrosion inhibitors were subjected to the Navy High Speed Bearing Test as described in Federal Test Method 331.1, and to the Pope Bearing Test as de-

Table I

| Grease Composition | Acid or Anhydride  | Reactants                   |                                                                                                                                              | Isocyanate | Base Oil | Thickener Conc, % wt | ASTM Penetration           |                          | ASTM Dropping Point, °F |
|--------------------|--------------------|-----------------------------|----------------------------------------------------------------------------------------------------------------------------------------------|------------|----------|----------------------|----------------------------|--------------------------|-------------------------|
|                    |                    | Phenylene Diamine           |                                                                                                                                              |            |          |                      | Unworked (P <sub>u</sub> ) | Worked (P <sub>w</sub> ) |                         |
| 1                  | Succinic anhydride | 4-Nitro-o-phenylene diamine | 70% mole C <sub>18</sub> H <sub>37</sub> NCO<br>30% mole C <sub>16</sub> H <sub>33</sub> NCO                                                 | A          | 15       | 250                  | 272                        | 510                      |                         |
| 2                  | Succinic anhydride | 4-Nitro-o-phenylene diamine | 70% mole C <sub>18</sub> H <sub>37</sub> NCO<br>30% mole C <sub>16</sub> H <sub>33</sub> NCO                                                 | C          | 18       | 238                  | 283                        | 513                      |                         |
| 3                  | Succinic anhydride | 4-Nitro-o-phenylene diamine | 100% mole C <sub>18</sub> H <sub>37</sub> NCO                                                                                                | B          | 14       | 290                  | 279                        | 514                      |                         |
| 4                  | Succinic anhydride | 4-Nitro-o-phenylene diamine | 100% mole C <sub>16</sub> H <sub>33</sub> NCO                                                                                                | B          | 11       | 260                  | 250                        | 502                      |                         |
| 5                  | Adipic acid        | 4-Nitro-o-phenylene diamine | 70% mole C <sub>18</sub> H <sub>37</sub> NCO<br>30% mole C <sub>16</sub> H <sub>33</sub> NCO                                                 | B          | 15       | 275                  | 298                        | —                        |                         |
| 6                  | Succinic anhydride | 4-Nitro-o-phenylene diamine | 63% mole C <sub>18</sub> H <sub>37</sub> NCO<br>27% mole C <sub>16</sub> H <sub>33</sub> NCO<br>10% mole C <sub>17</sub> H <sub>35</sub> NCO | A          | 14       | 279                  | 253                        | —                        |                         |
| 7                  | Succinic anhydride | 4-Nitro-o-phenylene diamine | 70% mole C <sub>18</sub> H <sub>37</sub> NCO<br>30% mole C <sub>16</sub> H <sub>33</sub> NCO                                                 | D          | 10       | 234                  | 285                        | —                        |                         |
| 8                  | Succinic anhydride | 4-Nitro-o-phenylene diamine | 70% mole C <sub>18</sub> H <sub>37</sub> NCO<br>30% mole C <sub>18</sub> H <sub>37</sub> NCO                                                 | E          | 15       | 253                  | 234                        | —                        |                         |
| 9                  | Succinic anhydride | 4-Nitro-o-phenylene diamine | 100% mole C <sub>12</sub> H <sub>25</sub> NCO                                                                                                | C          | 15       | 257                  | 290                        |                          |                         |

Base Oil A - Mineral lubricating oil having a viscosity of 500 SSU at 100°F.

Base Oil B - Mineral lubricating oil having a viscosity of 70 SSU at 210°F.

Base Oil C - Oligomerized alpha-olefin synthetic hydrocarbon oil having a viscosity of 7.7 centistokes at 210°F.

Base Oil D - Mineral lubricating oil having a viscosity of 430 SSU at 100°F.

Base Oil E - Mixture of hexadecyl isostearate and dimer acid esters.

scribed in Federal Test Method Standard 791a, Method 333. The bearing life in these tests is expressed in hours and represents the length of time until bearing failure occurred. Test results are recorded in the following table.

Table II

| Test Procedure                                                     | Grease <sup>1</sup><br>Composition 1 | Grease <sup>1</sup><br>Composition 6 |
|--------------------------------------------------------------------|--------------------------------------|--------------------------------------|
| Navy High Speed Bearing Test 300°F, 10,000 rpm, Bearing Life, hrs. | 3,388 <sup>2</sup>                   | 4,871                                |
| Pope Bearing Test, 350°F, Bearing Life, hrs.                       | 405 <sup>2</sup>                     | —                                    |

<sup>1</sup>Includes 1% wt. phenyl-alpha-naphthylamine, 0.5% Oronite 250 (dilauryl selenide), 1% wt. sodium sebacate and 0.03% wt. 3-amino-1,2,4-triazole.

<sup>2</sup>Average of two runs.

## EXAMPLE IV

Other dibenzimidazole-diurea thickeners and greases in accordance with the invention include those indicated in the following table.

Table III

| Grease<br>Com-<br>po-<br>sition | Reactants                                         |                                         |                                                                                              |                          |
|---------------------------------|---------------------------------------------------|-----------------------------------------|----------------------------------------------------------------------------------------------|--------------------------|
|                                 | Acid or<br>Anhydride                              | Phenylene<br>Diamine                    | Monoisocyanate                                                                               | Base<br>Oil <sup>1</sup> |
| 10                              | 1,2-Cyclo-<br>hexane<br>dicarboxylic<br>anhydride | 4-Nitro-<br>o-pheny-<br>lene<br>diamine | 70% mole C <sub>20</sub> H <sub>41</sub> NCO<br>30% mole C <sub>12</sub> H <sub>25</sub> NCO | A                        |
| 11                              | Azelaic<br>acid                                   | 4-Nitro-<br>o-pheny-<br>lene<br>diamine | 70% mole C <sub>18</sub> H <sub>37</sub> NCO<br>30% mole C <sub>16</sub> H <sub>33</sub> NCO | A                        |
| 12                              | Dodecyl<br>succinic<br>anhydride                  | 4-Nitro-<br>o-pheny-<br>lene<br>diamine | 100% mole C <sub>22</sub> H <sub>45</sub> NCO                                                | B                        |
| 13                              | Phthalic<br>anhydride                             | 4-Nitro-<br>o-pheny-<br>lene<br>diamine | 75% mole C <sub>18</sub> H <sub>37</sub> NCO<br>25% mole C <sub>16</sub> H <sub>33</sub> NCO | E                        |

<sup>1</sup>See footnote to Table I.

## EXAMPLE V

During the preparation and testing of various greases based on the present thickening agents, it was found that the dibenzimidazole-diurea compounds of the invention exhibit quite remarkable oxidation inhibiting activity when employed in conjunction with alkyl phenol or aryl amine-type antioxidants, particularly di- or tri-alkyl phenols and phenyl naphthylamines. This beneficial effect is demonstrated by the results presented in Table IV which were obtained by subjecting samples

of a mineral base oil containing the concentrations of antioxidants and thickening agent indicated in the table to an Air Oxidation Test at 350°F. In this test 9 liters of air per hour pass through 100 g of the test sample to which is added 20 ppm of soluble iron. The emergent air, after removal of contaminants, is passed through an oxygen analyzer which records the oxygen content of the air. Using a reference air stream, the rate of oxygen uptake is calculated. The test result which is called an induction period is defined as the time in hours required for 1 millimole of oxygen to be absorbed by the sample. A sample temperature of 350°F was used in these tests.

Table IV

| Test<br>Procedure | Alkyl<br>Phenol<br>Anti-<br>oxidant <sup>1</sup> | Aryl<br>Amine<br>Anti-<br>oxidant <sup>2</sup> | Dibenzimidazole-<br>Diurea <sup>3</sup> | Air Oxida-<br>tion Test<br>Induction<br>Period, |                   |
|-------------------|--------------------------------------------------|------------------------------------------------|-----------------------------------------|-------------------------------------------------|-------------------|
| 15                | %wt                                              | %wt                                            | %wt                                     | hrs.                                            |                   |
| 20                | A<br>B<br>C                                      | 1.5<br>None<br>1.5                             | 1.5<br>None<br>1.5                      | None<br>1.0<br>1.0                              | 21<br>2<br>72, 86 |

<sup>1</sup>2,6-Di-tertiary-butyl-4-methyl phenol

<sup>2</sup>Ocetylated phenyl-alpha-naphthylamine

<sup>3</sup>Thickener of Grease Composition 1

I claim as my invention:

30 1. A dibenzimidazole-diurea compound corresponding to the formula:



45 wherein R<sub>1</sub> and R<sub>2</sub> are hydrocarbyl radicals having 6 to 30 carbon atoms and R<sub>3</sub> is a hydrocarbylene radical having from 2 to 20 carbon atoms.

2. The compound of claim 1 wherein R<sub>1</sub> and R<sub>2</sub> are aliphatic hydrocarbyl radicals having from 12 to 24 carbon atoms.

3. The compound of claim 2 wherein R<sub>3</sub> is an alkylene radical having 2 to 12 carbon atoms.

4. The compound of claim 3 wherein the R<sub>1</sub> and R<sub>2</sub> radicals have from 16 to 18 carbon atoms.

5. The compound of claim 4 wherein R<sub>3</sub> is ethylene and R<sub>1</sub> and R<sub>2</sub> are hexadecyl, octadecyl or heptadecenyl.

\* \* \* \* \*